

# United States Patent Office

2,860,966

Patented Nov. 18, 1958

1

2,860,966

## METHOD OF PRODUCING GROUP IV-A METALS

Charles D. Atkinson, Wilmington, Del., assignor to E. I. du Pont de Nemours and Company, Wilmington, Del., a corporation of Delaware

No Drawing. Application January 31, 1955  
Serial No. 485,287

6 Claims. (Cl. 75—84.5)

This invention relates to the preparation of metals from group IV-A of the periodic table and more particularly to novel methods for effecting their preparation. More specifically, it relates to titanium or zirconium metal production by reducing a halide of such metal, especially a chloride, with a reducing metal, such as magnesium, and under conditions which will prevent objectionable iron contamination of the metal product.

Titanium and zirconium metals can be prepared by reducing their halides, e. g., titanium tetrachloride or zirconium tetrachloride, with a molten reducing metal, such as magnesium. Among known reduction procedures therefor, those disclosed in U. S. Patent Nos. 2,205,854, 2,564,337, 2,647,826, 2,663,634, 2,567,838 can be mentioned. The goal in such preparation is to obtain a product having the greatest possible purity, and many precautions and strict manipulative procedures have been proposed and are resorted to in attempts at attaining that goal.

The production of a low iron contaminated metal from such reduction procedures is highly desirable because the purity of the sponge titanium or zirconium metal reaction product is an important factor in its ultimate usefulness. In titanium metal, iron is considered to be a strong beta former, but the beta phase is not very stable in the contamination range of less than .05% iron. Iron present in titanium metal is detrimental because difficulty is encountered in producing all alpha alloys and the stability of the beta phase is low in mixed or all beta alloys. The reactor apparatus and equipment used in such production is constructed of iron which often enters as an objectionable impurity into the metal product due to inadvertent corrosion and attack of the equipment. To obviate this, recourse to expensive reaction vessel liners, made up of a refractory metal such as molybdenum have been proposed. These liners shield the iron vessel from the reactants and reaction products and prevent the titanium metal product from reacting directly with the iron reaction vessel. Other types of liners have been proposed, such as a removable low carbon steel sheeting material which is shaped to conform to the internal surfaces of the reaction vessel and is provided with a tapping outlet through which metal halide reaction by-product can be removed during the reduction.

In utilizing these liner elements, it has been customary that their surfaces be carefully cleaned and polished before use to remove all oxide scale or other surface coating therefrom with a view to avoiding iron or other metal contamination of the end product. Thus, in the Bureau of Mines Publication, IC 7381, November 1946, the teaching appears that prior to the reduction, the inside surfaces of the reactor are carefully cleaned by pickling in dilute HCl, scraping, and a final polishing with emery. Again, in the Bureau's publication, RI 4519, August 1949, it is taught that in setting up the equipment for the reduction, the first step is to thoroughly clean and polish the internal surfaces of the reactor pot with a rotating sand disc to remove scale and then the under-

2

surfaces of the reactor lid are dried prior to polishing with a rotary iron brush. Obviously, prior workers have been convinced that iron oxide scale presence on equipment employed in the reduction operation detrimentally affected the quality of the titanium metal product derived in the reduction.

I have found, contrary to previous practice and understandings, that cleaning and polishing the internal surfaces of an iron containing reaction vessel or the protective liner element utilized therein is disadvantageous in the metal halide reduction operations referred to, and that rather than minimizing or preventing iron contamination of the metal product such pretreatment promotes and induces undesired iron contamination. My further discovery is that, quite unexpectedly, said contamination can be effectively prevented or minimized by carrying out the reduction operation within a reaction vessel or protective liner, the surfaces of which are coated with a relatively thin, protective layer of iron oxide.

It is among the objects of this invention, therefore, to provide an improved method for producing a relatively pure form of group IV-A metal, especially titanium or zirconium, in which objectionable iron contamination of the product is effectively avoided; to provide novel methods and means for obtaining such product and without recourse to the disadvantageous, expensive, and time-consuming reactor surface polishing and descaling operations considered essential heretofore; and to provide a novel reduction process from which increased yields of relatively pure titanium or zirconium metal can be readily obtained. Other objects and advantages of the invention will be evident from the ensuing description.

These and other objects can be attained in this invention which comprises preparing a metal from group IV-A of the periodic table by reducing a halide of said metal under an elevated temperature within a closed reaction vessel the internal surfaces of which are coated with a protective layer of iron oxide.

The invention will be described in its application to one preferred adaptation involving the preparation of titanium metal by reducing titanium tetrachloride with a pool of molten magnesium in a closed reactor maintained at temperatures ranging from about 750-1100° C. In such operation iron contamination can arise from two sources. Thus, when reaction conditions vary beyond the close control required in the process and reaction temperatures above a limit of say 950° C. prevail, contact between the titanium metal product and the iron induces objectionable alloying at such point of contact.

Both iron and titanium are soluble in liquid magnesium, with iron being about 13 times as soluble as titanium at 900° C. The iron over and above the amount that can precipitate the titanium in solution combines with the titanium sponge and diffuses into the titanium surface. Consequently, contamination can also arise from solution of the iron in the container by the liquid magnesium metal and reaction of the dissolved iron with the titanium product. The reaction of dissolved iron with the titanium appears to be continuous with the iron being removed from the reaction container and transferred to the titanium metal. It is to the prevention of this latter type of contamination that the present invention is principally directed.

In accordance with this invention and in opposition to prior procedures which utilize oxide-free iron in contact with the liquid magnesium, I employ an oxide coated reaction vessel or container, especially one having a mill scale type of coating over its internal surfaces. Such types of vessels and containers have been highly efficacious in preventing undesired iron contamination. For example, I utilize within the reactor a suitable open-ended removable liner or casing element made up of hot-

rolled low carbon steel, said element being shaped to the interior configuration of the reactor and having necessary inlet and outlet means for introducing reactants and withdrawing reaction by-products. Preferably, this secondary reaction vessel is made up of oxide-coated sheet steel material having a thickness of, say, from .01 to .4 inch and, since titanium or zirconium react with carbon at relatively high temperatures, a carbon content of only .02 to .3%. Its seam or seams can be welded or otherwise suitably secured by means of similar light material which allows the liner to be readily stripped from the sponge metal reaction product after withdrawal from the reactor. The upper limits of the liner within the reactor can terminate short of the limits of the vertical walls of the reactor and at a point above the level of the reactant mass formed within the reactor. Its base portion can be provided with a restricted, downwardly-extending neck or outlet portion to conform to a discharge outlet coaxially arranged with the main reactor outlet. Suitable securing and lug element means can be provided on said liner adapted to retain it within the reactor and facilitate its handling, removal and replacement within the reactor.

In operation, the liner is positioned within the reactor and a sufficient charge of reducing metal, such as magnesium, is then introduced therein. The reactor is then covered in secured, air-tight relationship, and an argon or other suitable rare inert gas atmosphere is provided and maintained therein from a source of supply and until pressure conditions within the reactor are maintained in suitable, adjusted extent. Heat is then applied to the reactor by suitable furnacing or electrical heating means to melt the magnesium and maintain the reactor at temperatures ranging from about 750-1100° C. Upon reduction of the magnesium to molten state, liquid titanium tetrachloride is introduced at a controlled rate into the reactor, is immediately vaporized therein and reacts with the magnesium to form free titanium metal sponge. This secures itself to, bridges across the liner and builds up therein for subsequent removal with the liner for recovery. The released chlorine forms magnesium chloride with the reducing metal. This settles to the bottom of the reactor and flows downwardly into its bottom outlet for withdrawal, as desired from the system. Upon completion of the desired reaction, the liner or casing element together with its contained titanium metal reaction product is subjected to conventional purification treatment. The purified sponge metal is then recovered from the casing by stripping the latter therefrom, and can be formed into ingots or briquettes and fabricated into the desired metal or alloy product.

To a clearer understanding of the invention, the following illustrative example is given which is not to be construed as limiting the invention:

*Example*

The reduction apparatus used comprised an externally-heated, cylindrical, nickel-bearing steel reaction vessel having a 12" internal diameter and a height of 20". Within the reaction chamber of this vessel a removable, open-ended hot-rolled mill scale oxide coated low carbon (.05%) sheet steel liner having a .06" thickness, a diameter of 11½", and a height of 19" was fitted. This liner was shaped to conform to the internal configuration of the reaction vessel and was equipped, as was the vessel, with a bottom discharge spout arranged in coaxial relationship with a bottom inlet into the vessel. The reactor was maintained at a temperature of 850° C. by means of an external heater after all reactor inlets were sealed against the atmosphere, and an argon atmosphere was maintained therein. 15 lbs. of solid magnesium metal, previously charged into the retaining, protective liner, were then melted. Liquid titanium tetrachloride was then introduced into the reactor via an inlet in its upper portion and onto the surface of the molten magnesium. Such introduction was effected at a rate of about 20 lbs. per hour.

5 The titanium tetrachloride liquid immediately vaporized by the contained heat of the reactor and was thereupon reduced by the molten magnesium. Magnesium chloride formed in the process settled to the reactor bottom to flow through its descending coaxial disposed discharge spout and into a sealed cup disposed over the discharge outlet for said spout. Due to the cooler state of said outlet, the chloride cooled and solidified within the spout and its associated sealed cup to effectively prevent further by-product chloride discharge from the reactor. Titanium metal sponge formed within the liner bridged across and built up therein between its walls. Magnesium chloride by-product was drained from the reactor by remelting the frozen mass in the seal cup to allow the molten salt to flow therefrom and materially reduce titanium metal sponge contamination. When essentially all of the reducing metal had been consumed by the reaction and magnesium chloride tapped off, the equipment was cooled and the liner, together with its contained titanium metal sponge, was lifted out of the reactor and conveyed to a final purification stage of the system in which vacuum distillation equipment was effected at about 975-1000° C. In this latter operation any remaining magnesium chloride or other contaminants in the sponge were removed. Upon cooling the purified charge, the liner was easily peeled away from the titanium sponge, the latter being then ready for melting, casting or other conventional forms of treatment or fabrication.

30 An identical operation to the above was carried out except that the steel liner used consisted of one according with prior practice, i. e., previous to use it had been pickled, cleaned and dried, and then buffed and polished with a wire wheel until bright and oxide free.

35 Samples of each of these runs were taken and analyzed for iron contamination with the following results: the titanium resulting from use of the hot rolled oxide steel liner contained 0.23% iron, while the titanium from the pickled oxide free steel liner analyzed 0.36% iron. The latter is unacceptable as highest specification grade commercial titanium metal whereas the product from the oxide coated liner operation was wholly suitable for and met highest specification grade requirements.

40 Although described as applied to certain specific and preferred embodiments, the invention is obviously not restricted thereto. While magnesium comprises a preferred type of reducing metal, other metal reducing agents can also be used. Generally, use is contemplated of any reducing metal which is more electropositive than the preferred titanium or zirconium metal under production. 45 In addition to magnesium alkali and alkaline earth metals, including calcium, barium, strontium, sodium, potassium or lithium, can be employed. These are molten at 750° C. or higher, have relatively low specific gravities, and form a liquid halide as a by-product in the reduction reaction, to enable ready separation and removal of by-product halide from the metal.

50 As already indicated, the two metals preferred for production in this invention comprise titanium and zirconium. Generally, however, any group IV-A metal may be prepared hereunder, including titanium, zirconium, hafnium, etc. In such production, any of the halides of said metals may be employed, particularly those in which the halogen component has an atomic number greater than 9, i. e., chlorine, bromine, or iodine. The chlorides 55 of said metals, especially  $TiCl_4$  and  $ZrCl_4$ , are particularly useful herein and are therefore preferred for employment. The iodides and bromides of said metals are solids at room temperature, and while utilizable herein, are economically unattractive for use because of their relatively high cost.

55 The only major difference between the preferred titanium and zirconium producing processes is that when employing the tetrachlorides at atmospheric pressures, zirconium tetrachloride is a solid which sublimes at about 300° C., while titanium tetrachloride is a liquid at be-

between  $-30^{\circ}$  C. and  $136.4^{\circ}$  C. Since it is easier to admit gaseous zirconium chloride to the reaction chamber than the same compound in the solid state, one may readily elect to heat the reactant material prior to use in order to admit it to the system in a fluid or gaseous state. Thus, the chosen method of addition of the zirconium chloride may be different. Aside from this, these reactants may be added in any desired form, e. g., as solids, liquids, or vapors. If added as liquids or solids, they volatilize upon introduction into the heated reactor.

In my invention, magnesium is, as noted, the preferred reducing agent. During the reduction reaction and at least in the initial stages thereof, the magnesium exists as a liquid pool within the liner. The initial charge of magnesium can be added as solid ingots, bars, chips and melted in the liner, or it may be added in liquid state to the liner before initiating the reaction. Obviously, additional amounts of magnesium can be added during the reaction, either in the solid or the liquid state.

During the reduction the rate of reaction and the pressure prevailing within the reactor can be readily controlled by recourse to a neutral or inert atmosphere. While argon comprises a preferred form of protective gas, other inert gaseous elements of the group O of the Periodic System, such as helium or neon, or mixtures thereof, can be used. In employing the argon, a substantial partial pressure of such gas is maintained within the reactor during the reaction. This is adjusted to 760 mm. or higher during the tapping operation to avoid air influx and while the contents of the vessel are at or above the melting temperature of the metal halide reaction product. Alternatively, atmospheric or pressures above atmospheric (say, from 1-3 atmospheres or higher) can be employed, if desired.

The term "oxide scale" as used herein refers generally to the chemical compounds of iron and oxygen formed on the surface of steel by exposure to air while the metal is at an elevated temperature. Specifically, it comprises the oxidized surface of the steel produced during heating or working and during hot working. Hence, the oxide produced on a steel surface in hot rolling processes is known as mill scale. Chemical compounds thus formed comprise the various iron oxides,  $FeO$ ,  $Fe_2O_3$  and  $Fe_3O_4$ . The mechanism whereby mill scale forms is generally considered to be of a dynamic nature whereby alternate formation and reduction of the higher oxides of iron occur.  $Fe_2O_3$  is formed first and then reduced successively to  $Fe_3O_4$  and  $FeO$  by the availability of the iron during progress from the outer surface towards the iron center. The layer next to the steel,  $FeO$ , constitutes about 85% of the scale thickness;  $Fe_3O_4$ , the intermediate layer, about 10-15%; and  $Fe_2O_3$  the outer layer, about 1/2-2%. This scale exists on the hot rolled sheet steel product as it leaves the mill.

Oxide coatings can be produced on cold-rolled or pickled metal products by surface conversion coatings, such as "blue annealing," steam-bluing, air-bluing, or Bariffing treatments. While these types of oxide protective coatings are utilizable, the economics involving their use for liner purposes may not be as favorable as with hot rolled steel, because the steel base, prior to the treatment has been carried through a hot-rolling, pickling and possibly cold rolling operation.

While I prefer to employ a removable form of hot-rolled sheet steel protective liner, it will be evident that the liner element can be fixed or stationary within the reactor and form a component part thereof. Also, it is obvious that the oxide coating can be suitably applied to and formed directly on the internal surfaces of a steel reactor shell should use of a liner element be dispensed with. Thus, prior to use, such surfaces can be subjected to suitable oxidation treatment under elevated temperatures, conditions which will form thereon the desired protective oxide scale coating.

I claim as my invention:

1. A process for preparing a metal from group IV-A of the periodic table selected from the group consisting of titanium, zirconium and hafnium which comprises reducing a halide of said metal selected from the group consisting of a chloride, bromide and iodide with a reducing metal selected from the group consisting of alkali and alkaline earth metals, effecting said reduction under an elevated temperature ranging from  $750-1100^{\circ}$  C.
- 5 10 15 20 25 30 35 40 45 50 55 60 65 70 75
2. A method for producing titanium metal which comprises reducing a titanium halide selected from the group consisting of a chloride, bromide and iodide under an elevated temperature ranging from  $750-1100^{\circ}$  C. with magnesium within a closed reaction vessel the internal surfaces of which are coated with an adherent protective layer consisting essentially of iron oxide selected from the group consisting of  $FeO$ ,  $Fe_2O_3$ ,  $Fe_3O_4$ , and mixtures thereof, said layer constituting the only vessel contact with the reactants and reaction products during the reduction, and thereafter purifying and recovering the titanium metal product.
3. A method for producing zirconium metal which comprises reducing a zirconium halide selected from the group consisting of a chloride, bromide and iodide under an elevated temperature ranging from  $750-1100^{\circ}$  C. with magnesium within a closed reaction vessel the internal surfaces of which are coated with an adherent protective layer consisting essentially of iron oxide selected from the group consisting of  $FeO$ ,  $Fe_2O_3$ ,  $Fe_3O_4$ , and mixtures thereof, said layer constituting the only vessel contact with the reactants and reaction products during the reduction, and thereafter purifying and recovering the zirconium metal product.
4. A process for producing titanium metal which comprises reducing at a temperature of from  $750-1100^{\circ}$  C. titanium tetrachloride with molten magnesium within a closed reaction vessel and a sheet steel liner having an adherent oxide coating for said vessel consisting essentially of iron oxide selected from the group consisting of  $FeO$ ,  $Fe_2O_3$ ,  $Fe_3O_4$ , and mixtures thereof, said coating constituting the only vessel contact with the reactants and reaction products during the reduction, upon completion of the reduction reaction removing said liner with its contained titanium metal product from said vessel and subjecting the same to purification treatment, and upon completion of said purification, recovering the purified titanium metal product from said liner.
5. A process for producing titanium metal comprising reducing at a temperature of from  $750-1100^{\circ}$  C. titanium tetrachloride with molten magnesium within a closed reaction vessel and a removable hot rolled mill scale oxide-coated steel liner, the mill scale oxide coating consisting essentially of iron oxide selected from the group consisting of  $FeO$ ,  $Fe_2O_3$ ,  $Fe_3O_4$ , and mixtures thereof and which constitutes the only vessel contact with the reactants and reaction products during the reduction, upon completion of the reduction reaction removing said liner and its contained titanium metal product from said vessel and subjecting said product to vacuum distillation purification treatment within said liner, and subsequent to completion of said purification stripping said liner from the purified metal to effect recovery of the latter.
6. A process for producing zirconium metal comprising reducing at a temperature of from  $750-1100^{\circ}$  C. zirconium tetrachloride with molten magnesium within a closed reaction vessel and a removable hot rolled mill scale oxide-coated steel liner, the mill scale oxide coating

consisting essentially of iron oxide selected from the group consisting of  $FeO$ ,  $Fe_2O_3$ ,  $Fe_3O_4$ , and mixtures thereof and which constitutes the only vessel contact with the reactants and reaction products during the reduction, upon completion of the reduction reaction removing said liner and its contained zirconium metal product from said vessel and subjecting said product to vacuum distillation purification treatment within said liner, and subsequent to completion of said purification stripping said liner from the purified metal to effect recovery of the latter.

References Cited in the file of this patent

UNITED STATES PATENTS

- 2,205,854. Kroll ----- June 25, 1940  
 2,607,674. Winter ----- Aug. 19, 1952

OTHER REFERENCES

Evans: Corrosion of Metals, pp. 229-231; publ. 1926  
 by Ed. Arnold & Co., London.

Rawdon: Protective Metallic Coatings, pp. 53-54; publ. 1928 by The Chem. Catalog Co., Inc., New York.

Protective Coatings for Metals, by Burns et al. pp. 15-22; publ. 1939 by Reinhold Publ. Corp., New York.

5 The Electrochem. Soc. Preprint, 78-11, October 7, 1940, pp. 161-172.

Metal-Industry, May 16, 1947, pp. 363-364.

Metal Progress, February 1949, pp. 188-190.

Production of Ductile Titanium, by Wartman et al.

10 Bureau of Mines R. I. 4519, publ. August 1949 by Bureau of Mines, D. C. Entire report 37 pages. Fig. 2 and pages 6 and 24 pertinent; however, entire report relied upon.

Modern Metals, vol. VIII, No. 1, February 1952, pp. 15 29-31.

15 J. of the Electrochem. Soc., vol. 101, No. 10, October 1954, pages 507-513.